

## UNITED STATES PATENT OFFICE

2,527,334

MINERAL LUBRICATING OIL CONTAINING  
ALKALI AND ALKALINE EARTH METAL  
SALTS OF ALKYLATED DIBENZOTHO-  
PHENE SULFONIC ACID

Frederick P. Richter and Everett W. Fuller, Woodbury, N. J., assignors to Socony-Vacuum Oil Company, Incorporated, a corporation of New York

No Drawing. Application June 24, 1947,  
Serial No. 756,812

8 Claims. (Cl. 252—33)

1

This invention relates to alkylated dibenzothiophene sulfonic acids, to metal salts thereof, and to a method for preparing the same. More particularly, the present invention is concerned with lubricating oil compositions improved by incorporating therein a small proportion sufficient to improve the properties thereof of one or more of the aforesaid compounds.

In accordance with the present invention, it has been discovered that dibenzothiophene can be alkylated under certain conditions by contacting the same with an alkyl halide in the presence of a Friedel-Crafts type catalyst to produce alkylated dibenzothiophenes.

It has further been discovered that the alkyl dibenzothiophene produced as described above can be sulfonated by contact with a suitable sulfonating agent, such as chlorosulfonic acid, concentrated sulfuric acid, oleum, and the like.

Still further, it has been discovered that metal salts of the alkylated dibenzothiophene sulfonic acid, produced as a result of the aforesaid reaction, can be prepared upon contacting said acid with an inorganic salt or hydroxide of the desired metal. It has been further found that certain of said metal salts, notably those of the alkali and the alkaline earth metals, are useful as mineral oil additives and, more particularly, are effective as detergents in motor lubricating oils.

The compositions of this invention are prepared by using as a starting material substantially pure dibenzothiophene or a crude product which contains a major proportion of dibenzothiophene. This starting material is alkylated in accordance with the present invention by bringing the same into contact with an alkyl halide and a Friedel-Crafts catalyst, preferably in the presence of an inert organic solvent such as Stoddard's solvent.

The orientation of the alkyl group in dibenzothiophene has not been established with certainty. Indications are, however, that when only one hydrogen in each molecule of dibenzothiophene is replaced by an alkyl radical, the entering alkyl group occupies the 2- or 3-position and that when two hydrogens are replaced with alkyl groups, the entering radicals occupy the 2- and 8-positions or the 3- and 7-positions. The orientation, however, does not appear to be of too great significance in the practical synthesis of oil additive compositions prepared from the dibenzothiophenes so alkylated.

The initial ratio of alkyl halide to dibenzothiophene can be varied over wide limits and the degree of alkylation thus controlled to yield

2

mono-, di-, and polyalkylated dibenzothiophenes. Generally, however, a ratio of 1 to 3 gram atoms of halogen, as combined in the alkyl halide, per mole of dibenzothiophene has been found to be preferable. Alkylating agents of lower halogen content tend to result in a reduced yield of the desired alkyl dibenzothiophene, while those of higher halogen contents, as a general rule, give no added advantages and result in undue consumption of the alkyl halide. Mono- and di-alkylbenzothiophenes accordingly represent preferred embodiments of the invention.

It has been established, in accordance with this invention, that the temperature at which alkylation of dibenzothiophene is effected is a critical feature of the reaction. At temperatures below about 20° C., the alkylation reaction becomes so sluggish that the yield of desired product is practically nil; while at temperatures above about 20° C., a tar formation becomes predominant, causing a substantial decrease in the yield of desired product. Accordingly, the temperature range of from about 20° C. to about 85° C. appears to be a critical factor in the successful alkylation of dibenzothiophene. Particular preference is accorded to temperatures in the range of from about 60° C. to about 85° C., since under these conditions the reaction was found to proceed at a faster rate, and consequently as a practical matter, to yield a greater amount of alkylated dibenzothiophene per unit time as compared with lower temperatures in the operable range.

The use of an inert organic solvent, while not absolutely necessary, has been found to be highly desirable in modifying the alkylation of dibenzothiophene, causing a substantial decrease in the formation of undesirable tar as the condensation reaction proceeds. Any of the commonly employed organic solvents which are inert under the conditions of reaction may be employed for this purpose. Representative solvents include Stoddard's solvent, carbon disulfide, and the like.

In general, the process described herein may be employed for the alkylation of dibenzothiophene with any alkyl halide. However, when the sulfonate metallic salts of the resulting alkylated dibenzothiophene are to be employed as oil additives, alkyl halides of sufficient carbon chain length to render the prepared compound soluble in petroleum oil are preferred. For this, as well as economical reasons, the use of alkyl halides of hydrocarbons in the paraffin wax range having from about 20 to about 30 carbon atoms represents a preferred embodiment of this invention. Such alkyl halides having molecular weights in

3

excess of about 250 and having more than about 20 carbon atoms in their molecules are well known. Chlorinated wax may be considered as a preferred example of such compounds and, in particular, those waxes in which the degree of chlorination has been so regulated that the final chlorinated wax generally contains between about 5 and about 15 per cent chlorine.

The alkylated dibenzothiophenes described above may, in accordance with this invention, be sulfonated by dissolving in a suitable solvent and adding thereto a sulfonating agent such as chlorosulfonic acid. Concentrated sulfuric acid, oleum, or the like may also be used for sulfonating and may be employed directly. The ratio of sulfonating agent to alkylidibenzothiophene may be varied over a wide range to yield products of various degrees of sulfonation. In general, however, a ratio of 1 to 2 moles of sulfonating agent per mole of alkylidibenzothiophene is preferred. The addition of sulfonating agent to the solution of alkylidibenzothiophene usually is conducted at ordinary room temperatures, that is, between about 15° C. and about 30° C. Upon final addition of the sulfonating agent, the mixture is suitably heated under reflux for a period to insure complete reaction. The solvent employed may then be recovered by distillation. The residue obtained from said distillation is an alkylidibenzothiophene sulfonic acid.

In order to prepare metallic salts thereof, the alkyldibenzothiophene sulfonic acid as prepared above is dissolved in a suitable solvent, such as a refined petroleum oil, and the solution of sulfonic acid is converted to the desired metal salt by simple neutralization thereof with a metal hydroxide, carbonate or other alkaline inorganic salt of the metal. Alternatively, synthesis of the desired metal salt may be accomplished by metathesis of an alkali metal sulfonate prepared by one of the above mentioned methods with an inorganic halide of the desired metal.

The temperature at which the metal salt of alkyldibenzothiophene sulfonic acid is prepared will generally be in the range of from about 50° C. to about 200° C. and preferably between about 85° C. and about 150° C. The reaction mixture is maintained at an elevated temperature in the above range until all of the water of reaction is removed. During this operation, it is desirable but not necessary to bubble an inert dry gas such as nitrogen through the mixture in order to hasten the removal of said water. The resulting mixture is then suitably filtered through a clarifying agent, such as a filtering clay, to yield a petroleum oil solution of a metal alkyldibenzothiophene sulfonate.

The above described procedure may be employed in synthesizing any of the metal salts having the general formula:



where R is an alkyl radical, R' is selected from the group consisting of hydrogen and an alkyl radical and M is one equivalent of a metal. More specifically, where the metal salts are intended for use as additives in petroleum oils, M will represent an alkali or an alkaline earth metal and R will represent an alkyl radical in the paraffin wax range having a chain of 20 to 30 carbon atoms, and R' will likewise represent a hy-

1

drogen atom or an alkyl radical in the paraffin wax having a chain of 20 to 30 carbon atoms.

The metal alkylbenzothiophene sulfonates described above have been found to be particularly useful in lubricating compositions where they behave as detergents in maintaining the cleanliness of an engine.

These materials may be incorporated in any lubricating composition ranging from gasoline and kerosene to heavy gear oil, petroleum wax, and petrolatum. They may also be used with similar lubricating compositions derived from other animal, mineral, or vegetable sources, or prepared synthetically. Such lubricating compositions may contain any other desired addition agent or combination of addition agents which may be added for the purpose of effecting the same improvement or other improvements in that composition. Ordinarily, the new compositions described above will be added to mineral oil fractions in amounts ranging from about 0.1 to about 5 per cent but may be added in amounts up to 10 per cent in some instances. Those of the new products which are sufficiently soluble in oil may be marketed in the form of oil concentrates, in which the percentage of the new products is greatly in excess of that which is desired in the final lubricating composition, for example, quantities up to about 50 per cent by weight.

Further details and advantages of this invention will be apparent from the following illustrative examples:

*Example 1*

Petroleum wax of A. S. T. M. melting point of 125° F. was chlorinated by introducing chlorine gas at about 100° F. until 12 per cent by weight of chlorine was adsorbed therein. 596.6 parts by weight of the chlorowax so obtained were slowly added to a mixture of 184 parts by weight of dibenzothiophene, 596.6 parts by weight of Stoddard solvent, and 30 parts by weight of anhydrous aluminum chloride maintained at a temperature of 60° C. The temperature was allowed to gradually rise during the addition of the chlorowax to 75-85° C., in which range it was held during the alkylation. The mixture was agitated for a period of 4½ hours in this temperature range, after which time the active evolution of hydrogen chloride had practically ceased. To the cooled alkylation mixture, 500 volumes of 20 per cent aqueous hydrochloric acid were slowly added and the resulting mixture was heated to a temperature of 100° C. to hasten the separation of the mixture into organic and aqueous layers. After said separation was effected, the mixture was cooled and the aqueous layer was drawn off and discarded. The remaining organic layer was washed with water, filtered, and the solvent distilled off under vacuum. The dark green residue consisted of 706 parts by weight of a diwaxdibenzothiophene having a sulfur content of 4.1 per cent, the calculated sulfur content being 4.0 per cent.

Two hundred parts by weight of the diwaxdi-benzothiophene as prepared above were dissolved in 400 volumes of chloroform. Forty-one and two tenths parts by weight of chlorosulfonic acid were added dropwise to the resulting solution at room temperature. When the addition of sulfonating agent was complete, the mixture was heated under reflux for a period of 2½ hours to complete the reaction. The chloroform was then recovered by distillation and the residue was

## 5

Identified as a diwaxdibenzothiophene sulfonic acid having a neutralization number of 81, the theoretical neutralization number being 82.

## Example 2

The diwaxdibenzothiophene sulfonic acid as prepared in Example 1 was diluted with 400 parts by weight of an SAE 30 grade solvent-refined petroleum oil and 97 parts by weight of barium hydroxide octahydrate were added. The resulting mixture was held at a temperature of 85° C. for a period of 1 hour, raised gradually to 100° C. for 1 hour and finally increased to 150° C., where it was held until all of the water in the reaction mixture had been removed. This required maintaining the reaction mixture at the temperature of 150° C. for an additional hour. During this operation a steady stream of dry nitrogen gas was passed through the mixture in order to facilitate the removal of the water. The resulting hot oil solution was then filtered through Hi-Flo (a clay of the activated montmorillonite type represented by the ideal formula:



wherein  $n$  is an integer). The filtrate obtained from said filtration consisted of a petroleum oil solution of barium diwaxdibenzothiophene sulfonate having a barium content of 4.1 per cent and a sulfur content of 2.6 per cent.

## Example 3

The diwaxdibenzothiophene sulfonic acid prepared as in Example 1 was reacted with magnesium hydroxide, in the same manner as described under Example 2, for the preparation of the barium salt. The resulting product was an oil solution of the magnesium salt of diwaxdibenzothiophene sulfonic acid. It analyzed to give 1.1 per cent magnesium, the calculated magnesium content being 1.0 per cent.

## Example 4

A mixture consisting of 230 grams of a diwaxdibenzothiophene sulfonic acid, 23 grams of sodium hydroxide dissolved in 200 c. c. of methanol and 400 grams of a solvent-refined SAE 30 grade motor oil was heated under reflux with efficient stirring for 2 hours. The methanol and water of reaction were then removed by distillation with a steady stream of dry nitrogen gas passing through the mixture until the temperature reached 150° C. Final traces of methanol and water were removed by maintaining the temperature of the mixture at 150° C. with a current of dry nitrogen gas passing therethrough. The resulting hot oil solution was passed through a filtering clay at a temperature of about 95-100° C. in order to remove unreacted sodium hydroxide and other insoluble impurities. The product so obtained consisted of 520 grams of a clear oil solution of sodium diwaxdibenzothiophene sulfonate containing 1.4 per cent sodium and 3.2 per cent sulfur.

The above described metallic salts are effective as detergents in motor lubricating oils, as is demonstrated by the following test: Blends were made in a SAE 30 grade solvent-refined motor oil containing 0.75 per cent by weight of an antioxidant additive, consisting of the reaction product of pinene and phosphorus pentasulfide similar to that described in Example 3 of U. S. Patent

## 6

2,381,377. The following blends were prepared:

- A. Oil plus 0.75 per cent antioxidant.
- B. Oil plus 0.75 per cent antioxidant plus 5 per cent of the above described barium diwaxdibenzothiophene sulfonate.
- C. Oil plus 0.75 per cent antioxidant plus 2 per cent of the above described magnesium diwaxdibenzothiophene sulfonate.
- D. Oil plus 0.75 per cent antioxidant plus 2 per cent of the above described sodium diwaxdibenzothiophene sulfonate.

These blends were run in a single cylinder Lauson engine for a period of 100 hours at a speed of 1825 R. P. M. The oil temperature was maintained at 225° F. and the jacket temperature at 350° F. The engine was inspected at 20, 60, and 100-hour periods and the appearance of the piston was rated on a scale of 100 for a clean piston and lower values for increasing amounts of discolorization, lacquer, and sludge deposits. The following results were obtained:

|    |         | Cleanliness Rating |         |          |
|----|---------|--------------------|---------|----------|
|    |         | 20 Hrs.            | 60 Hrs. | 100 Hrs. |
| 25 | Blend A | 57                 | 32      |          |
|    | Blend B | 76                 | 67      | 66       |
|    | Blend C | 81                 | 69      | 68       |
| 30 | Blend D | 74                 | 68      | 55       |

The above results show that the alkali and alkaline earth metal salts of diwaxdibenzothiophene sulfonic acid are effective additives in improving the characteristics of lubricating oils.

The above described lubricating compositions are, of course, merely illustrative of those contemplated by the present invention. Antioxidants other than the pinene-phosphorus pentasulfide reaction product may be used. Likewise, various other improving agents may be present in the oil blend, such as V. I. agents, pour point depressants, oiliness agents, and the like.

We claim:

45. 1. A lubricating oil composition that comprises a mineral oil fraction and a small proportion sufficient to improve the detergent properties thereof of an alkaline earth metal salt of an alkylated dibenzothiophene sulfonic acid in which the sulfonic acid radical is attached directly to a benzene nucleus, said acid having an alkyl group of between about 20 and about 30 carbon atoms.
50. 2. A lubricating oil composition that comprises a mineral oil fraction and a small proportion sufficient to improve the detergent properties thereof of an alkali metal salt of an alkylated dibenzothiophene sulfonic acid in which the sulfonic acid radical is attached directly to a benzene nucleus, said acid having an alkyl group of between about 20 and about 30 carbon atoms.
55. 3. A lubricating oil composition that comprises a mineral oil fraction and a small proportion sufficient to improve the properties thereof of a compound selected from the group consisting of the alkali and alkaline earth metal salts of an alkylated dibenzothiophene sulfonic acid in which the sulfonic acid radical is attached directly to a benzene nucleus, said acid having an alkyl group of between about 20 and about 30 carbon atoms.
60. 4. A lubricating oil composition that comprises a mineral oil fraction and a small proportion sufficient to improve the detergent properties thereof of a sodium salt of an alkylated dibenzothiophene sulfonic acid in which the sulfonic

acid radical is attached directly to a benzene nucleus, said acid having an alkyl group of between about 20 and about 30 carbon atoms.

5. A lubricating oil composition that comprises a mineral oil fraction and a small proportion sufficient to improve the detergent properties thereof of a magnesium salt of an alkylated dibenzothiophene sulfonic acid in which the sulfonic acid radical is attached directly to a benzene nucleus, said acid having an alkyl group of between about 20 and about 30 carbon atoms.

6. A lubricating oil composition that comprises a mineral oil fraction and a small proportion sufficient to improve the detergent properties thereof of a barium salt of an alkylated dibenzothiophene sulfonic acid in which the sulfonic acid radical is attached directly to a benzene nucleus, said acid having an alkyl group of between about 20 and about 30 carbon atoms.

7. A lubricating oil composition that comprises a mineral oil fraction and between about 0.1 and about 5 per cent by weight of a compound selected from the group consisting of the alkali and alkaline earth metal salts of an alkylated dibenzothiophene sulfonic acid in which the sulfonic acid radical is attached directly to a benzene nucleus, said acid having an alkyl group of between about 20 and about 30 carbon atoms.

zene nucleus, said acid having an alkyl group of between about 20 and about 30 carbon atoms.

8. A lubricating oil composition that comprises a mineral oil fraction and a small proportion less than 10 per cent by weight of a compound selected from the group consisting of the alkali and alkaline earth metal salts of an alkylated dibenzothiophene sulfonic acid in which the sulfonic acid radical is attached directly to a benzene nucleus, said acid having an alkyl group of between about 20 and about 30 carbon atoms.

FREDERICK P. RICHTER,  
EVERETT W. FULLER.

15 REFERENCES CITED

The following references are of record in the file of this patent:

UNITED STATES PATENTS

| 20 | Number    | Name       | Date          |
|----|-----------|------------|---------------|
|    | 1,471,150 | Dziewonski | Oct. 16, 1923 |
|    | 1,996,334 | Hessle     | Apr. 2, 1935  |
|    | 2,160,293 | Shoemaker  | May 30, 1939  |
| 25 | 2,361,805 | Wilson     | Oct. 31, 1944 |
|    | 2,418,894 | McNab      | Apr. 15, 1947 |

**Certificate of Correction**

Patent No. 2,527,334

October 24, 1950

**FREDERICK P. RICHTER ET AL.**

It is hereby certified that error appears in the printed specification of the above numbered patent requiring correction as follows:

Column 6, line 64, before the word "properties" insert *detergent*;  
and that the said Letters Patent should be read as corrected above, so that the same may conform to the record of the case in the Patent Office.

Signed and sealed this 8th day of May, A. D. 1951.

[SEAL]

THOMAS F. MURPHY,  
*Assistant Commissioner of Patents.*